

# UNITED STATES PATENT OFFICE.

JOHN WILLIAM BLAGDEN, OF MANNHEIM, AND RICHARD MÜLLER, OF EILENBURG,  
GERMANY, ASSIGNEES TO C. F. BOEHRINGER & SOEHNE, OF MANNHEIM-WALDHOF,  
GERMANY, A FIRM.

## ART OF PREPARING FATTY-ACID COMPOUNDS.

1,000,487.

Specification of Letters Patent. Patented Aug. 15, 1911.

No Drawing.

Application filed October 28, 1907. Serial No. 399,590.

To all whom it may concern:

Be it known that we, JOHN W. BLAGDEN and RICHARD MÜLLER, citizens of the British Empire and the German Empire, respectively, residing at Mannheim and Eilenburg, Saxon Prussia, Germany, respectively, have invented certain new and useful Improvements in the Art of Preparing Fatty-Acid Compounds; and we do hereby 5 declare the following to be a full, clear, and exact description of the invention, such as will enable others skilled in the art to which it appertains to make and use the same.

This invention relates to fatty compositions to be employed for the manufacture of candles, night-lights and the like and processes of making the same; and consists in high melting fatty compositions viz. ammonia derivatives of acid fatty bodies, and 10 in a process of making such derivatives comprising the treatment of acid fatty bodies with ammonia, and the subsequent removal of impurities, excess of solvent, fatty acid, etc., and a certain amount of the absorbed 15 ammonia and alteration of such treated bodies by exposure to conditions all as more fully hereinafter described and as claimed.

Very little is known as to the ammonia salts of the higher fatty acids, such salts 20 being generally described as soapy bodies which gradually decompose into ammonia and the original fatty acid. In our work upon these bodies we have found that these ammonia soaps by treatment under certain 25 regulated circumstances can be obtained as stable bodies useful in the arts; such bodies being of higher melting point than the original fatty acid, stable under atmospheric conditions and burning without evolution of 30 ammonia or other injurious gases. Such bodies are consequently well adapted for making candles and night-lights. They may also be used for making "solid spirit", solidifying petroleum and for other purposes 35 for which waxes are now employed.

On treating acid fatty bodies with ammonia, which is best done with the materials as dry as possible, soapy bodies are formed and these soapy bodies when freed from 40 excess of solvent, fatty acid or other impurity and carefully dried, lose ammonia, till permanent bodies are formed. These products do not correspond to any very definite chemical compound, the ratio between the

ammonia group and the fatty acid group 55 varying with the conditions of preparations, and though this ratio frequently corresponds to that of an acid salt, this is not always the case. If after removing impurities the drying be performed in a vacuum desiccator at 60 about 15° C. for some days, a product is obtained which is perfectly stable and unchanged in air.

Any of the commercial acid fatty bodies may be treated in the described manner 65 with the described advantages of raising the melting point and preparing more waxy bodies. Oleic acid, for instance, may be made solid and given a relatively high melting point. A preparation made in the described manner from liquid oleic acid and containing nitrogen equivalent to 2.85 per cent. of NH<sub>3</sub> showed a melting point of 56° C., while another, prepared under somewhat different conditions and containing nitrogen 70 equivalent to 3.88 per cent. of NH<sub>3</sub>, had a melting point of 60° C. On still further raising the nitrogen content to the equivalent of about 4.20 per cent. NH<sub>3</sub>, the product had a melting point of about 75° C. 75 Elaidic acid, which normally melts at about 33°, under the described treatment gave a product containing nitrogen equivalent to about 3.30 per cent. of NH<sub>3</sub> and of a melting point of about 70° C. 80

Stearic acid, melting at 65° C., under the described treatment gave a solid waxy product containing nitrogen equivalent to 3.80 per cent. NH<sub>3</sub> and melting at about 87°. Erucic acid, which melts at 32°, gave a 90 product with nitrogen corresponding to 3.60 per cent. NH<sub>3</sub> and a melting point of about 52° C. 85

The ammonia and the fatty acid should be brought together in a condition as dry as 95 possible since the presence of moisture tends to diminish the stability of the products and increases the difficulties of purification.

One convenient way of obtaining a typical product from oleic acid is to dissolve a suitable quantity of oleic acid in a hydrocarbon, such as petroleum and lead ammonia gas into the cooled solution until a certain proportion of the fatty acid is precipitated as a dry soap. About 200 cc. of liquid oleic acid 100 may be dissolved in 400 cc. of petroleum oil and dry ammonia gas passed in till no further precipitate forms. The precipitate is 105

then filtered off, freed from the solvent by pressing, etc., and dried to constant weight.

In the drying operation, the amount given by the stated quantities of materials may be exposed in thin layers on trays to a low temperature of about 15-25° C. for about 48 hours under a vacuum of 29 inches. The resulting product will contain nitrogen equivalent to about 3 per cent. ammonia, will be permanent in air and will form an excellent candle material, either alone or in admixture with ordinary fats and waxes. The same quantity of stearic acid treated in the same way will give a waxy product containing nitrogen equivalent to about  $3\frac{1}{4}$  per cent. ammonia and having a melting point of about 87° C.

The oleic acid product may be melted with 1 or 2 parts of stearin or other fats or waxes to give a good candle material.

In all the described products, the new fatty body obtained is of higher melting point than the original acid fatty body, is colorless where the original acid was colorless, is of a waxy consistency, is anhydrous or free from water, is permanent in air, burns without evolution of ammoniacal gases, and contains firmly combined nitrogen in amount less than would correspond to a neutral ammonia salt of the acid treated.

The compound may be obtained in the form of a white powder if the original substance is colorless. It is quite insoluble in ether and it may, therefore, be purified by washing with ether, thereby removing excess of acid.

It has heretofore been proposed to mix fats or fatty acids with ammonia under pressure and at high temperatures varying between 150° and 250° centigrade. Under these conditions only the amids can be produced and not the ammonia salts of the fatty acids. Our process, whose object it is to obtain such ammonia salts, is distinguished from the so proposed process by the fact that it is carried out at temperatures below 100° centigrade, that is, below the temperature at which glycerin is distilled in practice. Only under these conditions can our new product be obtained.

Having thus fully described our invention, what we claim is:

1. In the art of making fatty acid compounds, the process which consists in treating a fatty acid, at a temperature below 100° centigrade, with ammonia and subjecting the mixture thus formed to mechanical pressure to remove the excess of solvent or liquid impurities.

2. In the art of making fatty acid compounds, the process which consists in mixing a fatty acid, at a temperature below 100° centigrade, with ammonia, subjecting the mixture to mechanical pressure and also to evaporative conditions at a temperature below the distilling temperature of glycerin to eliminate the excess of solvent or of liquid impurities and a portion of the ammonia.

3. In the art of making fatty acid compounds, the process which consists in introducing dry ammonia gas into a cooled fatty acid and subjecting the resulting mixture to pressure and to evaporative conditions at a temperature below 100° centigrade.

4. The process which consists in dissolving a fatty acid in a hydrocarbon and cooling the resultant solution, treating the solution with ammonia gas, and subjecting this mixture to pressure, and then drying *in vacuo*, and at a temperature below 100° centigrade, to remove the excess of solvent or liquid impurities and free ammonia.

5. As a new composition of matter, the stable anhydrous compound of a fatty acid with ammonia, the nitrogen contained in said compound being less in amount than corresponds to a neutral salt of said acid, said compound being stable in the air, having a higher melting point than the component fatty acid and evolving no ammoniacal vapors on combustion.

6. As a new composition of matter, the combustible stable anhydrous compound of a fatty acid with ammonia, said compound having a higher melting point than the component fatty acid, evolving no ammoniacal vapors on combustion and insoluble in ether.

7. As a new composition of matter, the dry combustible stable anhydrous compound of a fatty acid with ammonia, said compound having a higher melting point than the component fatty acid, evolving no ammoniacal vapors on combustion and insoluble in ether and in which the percentage of ammonia is not raised when washing the compound with a solvent for fatty acid.

In testimony whereof we hereunto affix our signatures, each in the presence of two witnesses.

JOHN WILLIAM BLAGDEN.  
RICHARD MÜLLER.

Witnesses as to the signature of John W. Blagden:

Jos. H. LEUTE,  
N. R. SHANK.

Witnesses as to the signature of Richard Müller:

RUDOLPH FRICKE,  
SOUTIARD P. WARNER.